

## UNITED STATES PATENT OFFICE

2,646,367

## TRANSFER PAPER

Chester Davis and Ned A. Thacker, Dayton, Ohio,  
assignors to The National Cash Register Company,  
Dayton, Ohio, a corporation of Maryland

No Drawing. Application June 28, 1951;  
Serial No. 234,161

2 Claims. (Cl. 117—36)

1

This invention relates to a manifold sheet, and more particularly pertains to one having a transfer coating that is hydrophobic and which contains a colorless recording oil which carries a colorless color-reactant material. The oil is carried in a low polar wax binder. The sheet is for use on specially sensitized paper used as an under sheet and the recording oil is transferred to the under sheet in printing and writing operations in a manner similar to the way in which transfer of coloring material is made from a carbon transfer sheet onto an under sheet, except that in the sheet of this invention the wax is colorless and plays no part in causing a mark on the under sheet, the only color producing material being the color reactant carried in the oil. In making carbon transfer sheets which have a wax coating containing a colored dye or pigment, oil is sometimes used with the wax to plasticize it so that it will transfer better, but the oil plays no part in causing the colored mark, such being made by the colored wax. The fact that the wax, oil, and color-reactant carried by the oil, are all hydrophobic, renders the transfer sheet immune to the effects of humidity. The color reactants are so chosen as to need no moisture for the creation of color on the underlying sheet.

The sensitized under sheet with which the novel manifold sheet is intended to be used is sensitized by particles of acid-like, inorganic material, also colorless or nearly so in the finely divided state. Typical of such sensitizing pigments are attapulgite; sodium zeolite material; sodium zeolite material in which the natural sodium exchange ions have been replaced by the ions of hydrogen, nickel, copper, iron, zinc, mercury, barium, lead, cadmium, and potassium; halloysite; and magnesium trisilicate. These pigments in finely divided form, either singly or mixed, may be applied to the paper in a suitable paper coating binder material, such as paper coating starch, casein, or latex, the proportion of pigment to binder material being such that a large proportion of the surface area of the pigment particles is exposed for contact by the recording oil transferred thereto by the novel manifold sheet. The pigment materials mentioned are practically colorless and give the same effect and adhere to the paper as does ordinary paper coating clay. The sensitized receiving sheet is more fully described in United States Patent 2,548,364, which issued on the application of Green and Sandberg. The color reaction in which the oil-carried color-reactant takes part is a so-called adsorption color reaction in which the pig-

ment acts as an electron acceptor with reference to the color reactant material carried by the oil, and is an adsorbent with respect to such color reactant. The color reactant materials carried by the oil are aromatic double-bond organic compounds, normally colorless, which upon adsorption on the pigment are converted to a more highly polarized conjugated form, accompanied by the appearance of color. This color reaction phenomenon is also fully set forth in the patent to which reference has been made. Examples of the organic color reactant will be given in the description to follow.

Several of the most important features of the novel transfer sheet are that it may be handled without discoloring the hands. It may be rubbed onto an unsensitized surface without leaving a mark. It is immune to humidity and it has a clean colorless appearance which is strikingly different from ordinary carbon manifold transfer sheets heretofore known. The marks made on the sensitized under sheet requiring the presence, in adsorption contact, of the acid-like pigment for the appearance of color, will not come off onto the hands of a person who makes contact with the colored marks, any oil that is unused when rubbed off from the under sheet being colorless, and any of the reactant color-reactant material which may be desorbed from the receiving sheet losing its color and reverting to the original colorless state. It will be seen, therefore, that there are uses for the novel manifold sheet in which these characteristics are of great value as, for instance, in the field of sales books, in which a duplicate copy of a sales entry is made on the underlying sheet by means of a manifold transfer coating. The manifold sheet which constitutes the original entry will have on its back the transfer coating, but it is colorless, will not be rubbed off by wet hands, and may be safely placed with white merchandise without smudging such. Moreover, the copy on which the marks were made by the transfer coating may be safely placed with such white merchandise without discoloring it because, as has been said, the wax which may be accidentally rubbed off is colorless, or nearly so, and contains no colored material, all the color in the mark being in the color reactant which is absorbed and attached to the pigment particles which are found upon the receiving sheet. Again, in this respect, this manifold sheet differs from carbon paper in that the marks made by carbon paper may rub off the receiving sheet with the wax, carrying with it the coloring material, smudging whatever comes in contact therewith.

The novel manifold sheet may be kept in contact with the sensitized receiving sheet in stacks, as would be the case in a bound duplicating sales book, without the appearance of color on the under sheet by transfer of the oil thereto, the wax and oil system having been provided with such in mind.

This manifold sheet is not to be confused with the type of sheet shown in United States Patent 2,374,862, which issued on the application of Barrett K. Green, inasmuch as that patent showed a manifold sheet having a rupturable hydrophylic colloid film in which were dispersed discrete fluid inclusions of an oil which contained either a coloring material in the colored form or a color-reactant. That patent indicated as one of the useful color-reactant materials, the compound tetra-methyl-diamino-diphenyl-phthalide, which is commonly known as malachite green lactone, having the molecular formula 3,3 bis (p-dimethylaminophenyl) phthalide. That compound is also useful in the transfer coating of this invention, but it is carried in a wax binder and not in the form of liquid droplets in a hydrophylic binder, the wax being hydrophobic. Neither should the transfer coating or film of this invention be confused with the transfer coating set out in United States Patents 2,550,466 to 2,550,473 inclusive, which disclose a rupturable film containing droplets, the film being of a hydrophylic nature. In the patents to which reference was made, and which disclose a transfer coating consisting of a rupturable hydrophylic film containing droplets, the transfer coating was made by deposition on paper of an emulsion having an external phase which is dryable to form the rupturable film and an oil internal phase, carrying the color, which remains in the dry film as droplets. The external phase is a solution of hydrophylic colloid material in water and the coating dries to a film by evaporation of the water. In the manifold sheet of this invention the transfer film is applied as a hot melt coating which solidifies by cooling, and the oil is not contained in droplets but is combined with the wax as an intimate mixture of two hydrophobic materials.

The hydrophobic wax must be chosen so as not to have a tendency to coat over the active surfaces of the pigment particles, and the wax must hold a high content of the recording oil. Moreover, the wax must be of low polarity so as not to interfere with the color reactant, and it must be resistant to smudging action when resting on an underlying receiving sheet under moderate pressure. It will be appreciated that in marking and printing operations, the pressure per unit area is many times that which is obtained by mere stacking of the papers together. Another obstacle to be overcome is that the sensitizing materials on the underlying sheets are selected because of their adsorbent nature and hence they tend to draw out the oil from the transfer film in contact therewith and such film must be highly resistant to such adsorbent effect.

Therefore, it is an object of this invention to provide a manifold sheet having a transfer film including oil intimately mixed with a wax binder, said oil containing a colorless adsorbate color-reactant, for use on record material with a highly adsorbent pigment which causes the adsorbate to assume a distinctive color when in adsorption contact therewith.

Another object of the invention is to provide such a manifold sheet in which the film mate-

rials, including the wax, oil and color-reactant, are all hydrophobic materials.

A still further object of the invention is to provide such a system in which, by the addition of inert particle material thereto, the resistance of the transfer film to smudging is increased.

With these and incidental objects in view, the invention includes certain novel features and combinations of ingredients, a preferred form or embodiment of which is hereinafter described in detail.

#### General description

In the preferred embodiment of the invention, about 55%, by weight, of colorless oil containing the hydrophobic color-reactant is mixed with 45%, by weight, of wax. The percentage of oil with respect to the wax may vary from 25%, by weight, to 75%, by weight. The colorless oil with reactant is made up of 94%, by weight, of petroleum lubricating oil of a 200 seconds Saybolt viscosity, and 6%, by weight, of the color reactant which is made up of one-half crystal violet lactone and one-half benzoyl leuco methylene blue. The crystal violet lactone is 3,3 bis (p-dimethylaminophenyl) 6-dimethyl-amino phthalide, and may be made by the method disclosed in United States Patent Re. 23,024, which issued on the application of Clyde S. Adams. Crystal Violet Lactone has the following structure:



The benzoyl leuco methylene blue has the following structure:



55 The crystal violet lactone is an adsorption color reactant and immediately upon making contact with the pigment on the sensitized paper, as described, turns to a dark blue and the benzoyl leuco methylene blue when in contact with the 60 sensitizing pigment oxidizes, after a passage of some time, into a dark blue color, fortifying the crystal violet lactone color which is apt to fade after long exposure to light and air. The wax, comprising 45% of the mixture forming the coating, is itself a mixture of waxes, 4/9 being sugar cane wax, another 4/9 being fully refined paraffin wax, and 1/9 being Montan wax. The wax is heated until it is melted to a consistency where it can be readily stirred and the oil, with the color reactant therein, is added and the mixture thoroughly stirred until the ingredients are homogeneously integrated. This mixture, while still in the melted condition, is applied as a coating on paper in the same manner as wax-base carbon 70 paper coatings are applied, and to a comparable

thickness, 6 pounds of coating per ream of 36" x 48" being sufficient, although more or less may be applied. This coating is discernible on the paper, not by its color, but by the texture of the surface and its light reflecting qualities.

In a second embodiment of the invention 58%, by weight, of the colorless recording oil, is used with 22%, by weight, of Ouricury wax and 20% of fully refined paraffin wax, and this is used in the same manner as the mixture of the preferred embodiment.

In the third embodiment of the invention 55%, by weight, of the colorless recording oil is mixed with 45%, by weight, of Carnauba wax.

In a fourth embodiment of the invention 60%, by weight, of the colorless recording oil is used with 25%, by weight, of Ouricury wax and 15%, by weight, of montan wax. In this embodiment, the colorless oil is 75%, by weight, of the same kind of petroleum lubricating oil mentioned in the preferred embodiment, and 25%, by weight, of chlorinated diphenyl of a chlorine content of 65%. The color reactants may be used in the same amount as described for the preferred embodiment. The resinous character of the chlorinated diphenyl helps prevent smudge.

The wax may be modified by use of other resinous material than chlorinated diphenyl to increase smudge resistance, coumarone indene being suitable.

In a fifth embodiment, 50%, by weight, of the colorless recording oil of the preferred embodiment is mixed with 25%, by weight of montan wax, and 25%, by weight, of fully refined paraffin wax.

In all of the above embodiments, inert fillers to the extent of 5% to 15%, by weight, of the coating may be incorporated into the mixture to decrease the possibility of smudge when in storage contact with the sensitized paper with which it is to be used. Mineral fillers, such as titanium dioxide, calcium carbonate, and barium sulphate, are satisfactory, but hydrophobic carbethoxylated starch derivatives such as sold by the National Starch Company, under the name of "Dry-flo," have been found to be of exceptional merit.

Following are some hydrophobic color-reactants, among the many available, which may be used alone or substituted for the crystal violet lactone with the benzoyl leuco methylene blue, which have been previously specified:

(a) Xanthene-9,0-benzoic acid, 3,6-bis-diethylamino - 9 - p-nitroanilino - lactam, having the structure



and which turns from a normally colorless state to red on the sensitized record material.

(b) Michler's hydrol, which is, bis(p-dimethylaminophenyl) methanol, having the structure



and which turns from a normally colorless state to dark blue on the sensitized record material.

(c) Malachite green lactone, which is 3,3 bis(p-dimethylaminophenyl) phthalide, having the structure



which changes from its normally colorless state to green on sensitized paper.

(d) 3,3 bis(p-diethylaminophenyl) phthalide, having the structure



which changes from its normally colorless state to blue-green on sensitized paper.

(e) 3,3 bis(p-di-n-propylaminophenyl) phthalide, having the structure



which changes from its normally colorless state to deep green on sensitized paper.

As substitutes for the petroleum oil mentioned are the chlorinated or alkylated diphenyls having equivalent viscosity, hydrogenated terphenyls, diethyl phthalate and chlorinated paraffin. The following waxes may be used and are miscible with the specified colorless recording oil: Carnauba wax, Ouricury wax, Candelilla wax, vegetable fiber wax, Esparto wax, sugar cane wax, Montan wax, Ozokerite wax, Ceresin wax, Utah wax, micro-crystalline waxes having a melting point of between 170 degrees and 200 degrees Fahrenheit, and fatty-acid amides. Synthetic waxes such as hydrogenated castor oil and Montanic acid esters may also be used. These waxes may be compounded together to meet the requirements of hardness and smudge resistance required.

It will be evident from the foregoing that the novel manifold sheet may be made from many substances, and that the invention does not reside with the particular oils, waxes, and color reactants used, except for their characteristics of miscibility, hydrophobic nature, lack of color, and consistency for use as transfer materials useful in printing and writing.

While the embodiments of the invention herein described are admirably adapted to fulfill the objects primarily stated, it is to be understood

that it is not intended to confine the invention to the particular ingredients or embodiments herein disclosed, for the invention is susceptible of embodiment in various other forms.

What is claimed is:

1. A manifold sheet for use in conjunction with a copy-receiving sheet sensitized on the copy-receiving surface thereof with particles of inorganic clay-like material, said particles having acid-like adsorbent surfaces, including a base web; and a film on said web of a substantially colorless hydrophobic low polarity wax having mixed therein a substantially colorless atmospherically stable hydrophobic oil containing a substantially colorless hydrophobic double bond aromatic atmospherically stable adsorbate compound, which organic compound is converted to a more highly polar conjugated form accompanied by the appearance of a distinctive color therein when adsorbed on particles of inorganic clay-like ma-

5

10

15

20

terial which acts as an electron acceptor with respect to said organic compound on adsorption contact therewith, and the oil and adsorbate compound being 25% to 75% of the total weight of the film.

2. The sheet of claim 1 in which there is incorporated, with the wax, oil and color reactant, a hydrophobic finely divided filler material.

CHESTER DAVIS.  
NED A. THACKER.

References Cited in the file of this patent

UNITED STATES PATENTS

| Number    | Name   | Date          |
|-----------|--------|---------------|
| 2,040,075 | Brower | May 12, 1936  |
| 2,503,680 | Newman | Apr. 11, 1950 |
| 2,548,366 | Green  | Apr. 10, 1951 |
| 2,554,909 | Holik  | May 29, 1951  |